

April 25, 1939.

W. H. MELANEY

2,155,610

COMPOSITE ROLL

Filed July 19, 1938

2 Sheets-Sheet 1

Fig. 1



Fig. 2



Fig. 3



Fig. 4



Fig. 5



BY

INVENTOR.  
William H. Melaney  
William B. Jasper

ATTORNEY.

April 25, 1939.

W. H. MELANEY

2,155,610

## COMPOSITE ROLL

Filed July 19, 1938

2 Sheets-Sheet 2

Fig. 6



Fig. 7



Fig. 8



INVENTOR.

INVENTOR.  
William H. Melaney  
William B. Jagger

ATTORNEY.

## UNITED STATES PATENT OFFICE

2,155,610

## COMPOSITE ROLL

William H. Melaney, Pittsburgh, Pa.

Application July 19, 1938, Serial No. 219,995

2 Claims. (Cl. 22—206)

This invention relates to new and useful improvements in chilled or alloy rolls for metal rolling mills, more particularly to the method of making same, and it is among the objects thereof 5 to provide a method of making rolls for metal rolling mills of a composite metal to provide a chilled body surface for the face of the roll of a dense hard or tough metal and neck or journal portions of an easily machinable metal, whereby 10 the costly machining and grinding operations incident to the manufacture of such rolls by methods heretofore practiced are substantially reduced.

A further object of the invention is to provide 15 a composite metal roll in which the outer portions of the necks or bearings are constituted of prefabricated metal sleeves which are cast integrally with the main body of the rolls and which may be prepared in a manner to produce a fusion of 20 substantial portions of the neck or bearing portions with the metal forming the main body of the rolls.

Still a further object of the invention is the provision of a metal roll in which the working 25 body of the roll is cast of a tough or hard metal and in which the necks, bearings or driving portions are partially constituted by preformed sleeve castings and partially of poured metal of different characteristics than the preformed sleeve portions, the main body, the sleeve portions, and 30 the metal joining the sleeve and main body portions being integrally formed by casting.

These and other objects of the invention will 35 become more apparent from a consideration of the accompanying drawings constituting a part hereof in which like reference characters designate like parts and in which:

Fig. 1 is a vertical cross-sectional view of a 40 mold for casting rolls for metal rolling mills embodying the principles of this invention;

Fig. 2 a view partially in section and partially 45 in side elevation of a preformed sleeve which is adapted to be joined integrally with the neck portion of the roll;

Fig. 3 a vertical cross-sectional view of a preformed sleeve having the inner wall surface thereof provided with annular serrations;

Fig. 4 a transverse section taken along the lines 4—4, Fig. 1;

Fig. 5 a similar section showing a different 50 form of serrations;

Fig. 6 a vertical cross-sectional view of a mold for casting rolls embodying a modified form of the invention;

Fig. 7 a side elevational view of a neck of vary-

ing insert for use in the method of making rolls by the apparatus shown in Fig. 6; and

Fig. 8 a vertical cross-sectional view of the mold shown in Fig. 7.

With reference to Fig. 1 of the drawings, the 5 numeral 1 designates a metal mold having an interior matrix surface 2 corresponding to the contour of the main body portion of the roll to be cast, the metal mold quickly chilling the casting to a substantial depth to constitute a very 10 hard rolling surface, which is finished by a grinding or machining operation. The numeral 3 and numerals 4 and 5 designate mold sections or flasks for receiving sand 6, the top portion being molded to form a sink-head 7 and the bottom portion of the sand mold is gated to a down-runner 8 through which the metal is poured, the gate 9 being disposed to produce a tangential flow of metal which sets up a swirling motion to the molten metal as it enters the mold.

Numerals 10 and 11 constitute the neck or 15 bearing portions of the roll and the numerals 12 and 13 the wobbler ends. The neck portions 11 and 12 are formed of prefabricated sleeves 14, Figs. 2 and 3, the sleeve in Fig. 2 being provided 20 with serrations or flutes 14a as shown in Fig. 5, which are axially disposed and the serrations or flutes 15, Fig. 3, are of annular form. These neck portions may be pickled, machined, or sandblasted or otherwise prepared to clean the inner 25 surfaces and may be coated with a non-oxidizing or rust-preventing substance such as by galvanizing or zinc coating before placing them in the sand portions, as shown in Fig. 1.

In casting the roll, the metal forming the main 30 body portion of the roll designated by the numeral 16 is first poured into the down-runner 8 and enters the base of the mold, filling the matrix portion thereof to just above the top of wobbler 12, the sink-head portion 7 remaining empty of 35 metal. The metal thus initially poured into the mold is of a character suitable for the severe rolling operations to which the roll is subjected in rolling mill practice, and is chilled for a substantial depth along the metallic matrix portion 2 as heretofore explained.

A softer or more readily machinable metal is 40 then poured through the runner 8 to displace only the molten metal of the down gate and sprue. The same metal is then poured into the sink-head 7 to feed downwardly into the upper neck portion as the metal contracts in the main body portion of the roll for sinking purpose only.

When the metal is poured as described, it will 45 fuse or melt the serrated portions 14a and 15,

as the case may be, to effect an intimate welding of the preformed neck pieces with the adjacent cast or supporting body portion of the roll, it being obvious that the faces of the neck portions 13 may be otherwise prepared to promote the welding action of the molten metal with the preformed sleeve portions.

As shown in Fig. 2, the bottom neck portion 13 is provided with a gate 17 and by employing metal of the same or similar properties as that of which the neck pieces 13 are formed for the displacement of the metal from down gate and sprue only, initially poured to form the main body of the rolls, the gate 17 will be of the same material as the sleeve 13, so that the finished roll will have no hard spot on the finished surface of the neck or bearings.

In Fig. 6 of the drawings, neck or bearing sleeves 18 are provided with flanges 19 which extend into the matrix portion 2 of the mold in which the roll body is cast. Because of the swirling motion of the metal entering the bottom of the mold through the offset gate 17, it will form a meniscus as shown at 20 and 21, Fig. 6, all impurities of the metal accumulating in the depressed portion at 22 and 23. As the metal rises, the metal at the outer edge is free from impurities and when it reaches the level above the flange 19 of the insert that forms the neck or bearing of the roll, it will flow in the annular space 24. As it rises further, as shown near the top of the roll body matrix 2, the same meniscus effect is maintained so that pure metal will reach the annular space 24a between the flange 19 and the roll body matrix. Otherwise, the pouring of the metal through the down-gate is the same as described in connection with Fig. 1, the metal being filled to the top of the wobbler 12. It is then displaced by softer metal of the character of the neck sleeves 18 to an amount just sufficient to displace the metal in the gate 17 of the sleeve portion so that upon subsequent machining there will be no hard spots in the neck or bearing portion. The same grade of metal is poured into the sink-head 7 to feed into the top of the casting when shrinkage takes place.

In Figs. 6 and 8 I have shown the sleeve portions lined at 25 with sheet, copper, or other metal which may be coated with a flux so that when the molten metal is poured into the mold it will be welded or brazed with the metal of the sleeves 18 through the fusing action of the lining 25. This is an alternative method of bonding the cast metal with the preformed sleeve members to that employing the serrations or flutes of the sleeves shown in Figs. 2 and 3 of the drawings.

By employing the flanged sleeves as shown in

Fig. 6, the clear line of demarkation will result between the outer periphery of the flanges 19 and the metal in the annular grooves 24 which will be immediately apparent when the neck and roll portions are machined and/or ground after the casting operation.

Rolls cast as hereinbefore described have a main body portion 16 of a very hard or tough metal which may be finished by machining or grinding, whereas the neck portions 10 and 11 are of a softer material which may be readily machined to size without requiring the long tedious grinding or other slow machining operations to reduce said parts to their approximate finished dimensions as in the manner of conventional practice, the elimination of which results in a very substantial reduction in the cost of machining these rolls.

Although several embodiments of the invention have been herein illustrated and described, it will be evident to those skilled in the art that various modifications may be made in the details of construction without departing from the principles herein set forth.

I claim:

1. The method of making rolls for metal rolling mills and the like which comprises providing a mold consisting of a metallic matrix portion for casting the main body of the roll, sand portions adjacent to the metal body portion for casting the necks and wobblers of the roll and a down gate and sprue for one of the sand portions, placing sleeve portions of preformed metal in the sand portions of the molds to form the outer portions of the necks thereof, pouring molten metal in the bottom of the mold to form the main body of the roll, displacing said cast fluid metal from the down-gate and sprue of the mold by fluid metal of the character of the preformed sleeve portions, and pouring metal similar to the metal of the sleeve portions in the sink-head at the top of the mold to fill the void caused by shrinkage in the main body portion of the mold.

2. The method of making rolls for metal rolling mills and the like which comprises the steps of inserting prefabricated sleeve portions in a mold adjacent the main body chill, the sleeve portions having fluted inner surfaces constituting passages for the molten metal poured in the mold, pouring the metal for the main body portion into the mold to completely fill the mold in contact with the fluted surfaces of the prefabricated sleeve portions to thereby melt the fluted surfaces of the sleeve portions to produce a fusing of the molten metal with the metal of the prefabricated sleeve portions.

WILLIAM H. MELANEY.

CERTIFICATE OF CORRECTION.

Patent No. 2,155,610.

April 25, 1939.

WILLIAM H. MELANEY.

It is hereby certified that error appears in the printed specification of the above numbered patent requiring correction as follows: Page 1, second column, lines 32 and 33, strike out the words "such as by galvanizing or zinc coating"; and that the said Letters Patent should be read with this correction therein that the same may conform to the record of the case in the Patent Office.

Signed and sealed this 1st day of August, A. D. 1939.

(Seal)

Henry Van Arsdale,  
Acting Commissioner of Patents.